



US006238148B1

(12) **United States Patent**  
Taniuchi et al.

(10) **Patent No.:** US 6,238,148 B1  
(45) **Date of Patent:** May 29, 2001

(54) **CEMENTED CARBIDE CUTTING TOOL**

(75) Inventors: **Toshiyuki Taniuchi, Kazuki Okada,**  
both of Ibaraki-ken; **Kazuhiko**  
**Akiyama**, Ohmiya, all of (JP)

(73) Assignee: **Mitsubishi Materials Corporation,**  
Tokyo (JP)

(\*) Notice: Subject to any disclaimer, the term of this  
patent is extended or adjusted under 35  
U.S.C. 154(b) by 0 days.

(21) Appl. No.: **09/256,218**

(22) Filed: **Feb. 24, 1999**

(51) **Int. Cl.<sup>7</sup>** ..... C22C 29/00; B23P 15/28  
(52) **U.S. Cl.** ..... 407/119; 407/118  
(58) **Field of Search** ..... 407/118, 119

(56) **References Cited**

U.S. PATENT DOCUMENTS

|           |   |         |                   |         |
|-----------|---|---------|-------------------|---------|
| 1,728,909 | * | 9/1929  | Schroter          | 407/119 |
| 4,708,037 | * | 11/1987 | Buljan et al.     | 407/119 |
| 4,950,328 |   | 8/1990  | Odani et al.      | .       |
| 5,009,705 | * | 4/1991  | Yoshimura et al.  | 407/119 |
| 5,230,729 |   | 7/1993  | McCandlish et al. | .       |
| 5,372,797 |   | 12/1994 | Dunmead et al.    | .       |
| 5,529,804 |   | 6/1996  | Bonneau et al.    | .       |
| 5,624,766 | * | 4/1997  | Moriguchi et al.  | 407/119 |
| 5,651,801 | * | 7/1997  | Monroe et al.     | 51/309  |
| 5,880,382 | * | 3/1999  | Fang et al.       | 51/309  |
| 5,908,478 | * | 6/1999  | Wood              | 51/309  |

5,921,330 \* 7/1999 Sue et al. ..... 51/309  
5,955,186 \* 9/1999 Grab ..... 407/119  
5,984,593 \* 11/1999 Bryant ..... 407/119

FOREIGN PATENT DOCUMENTS

|          |   |        |      |         |
|----------|---|--------|------|---------|
| 3-43113  |   | 2/1991 | (JP) | .       |
| 5-69204  | * | 3/1993 | (JP) | 407/119 |
| 10-53831 | * | 2/1998 | (JP) | .       |

\* cited by examiner

*Primary Examiner*—A. L. Wellington

*Assistant Examiner*—Erica Egenbright

(74) **Attorney, Agent, or Firm**—Oblon, Spivak, McClelland,  
Maier & Neustadt, P.C.

(57) **ABSTRACT**

In a cemented carbide cutting tool made of a tungsten carbide-based alloy comprising 8 to 13 percent by weight of Co and 0.1 to 3 percent by weight of Cr as constituents for forming a binding phase, the balance being tungsten carbide as a constituent for forming a dispersing phase and incidental impurities, the rate of the dispersing phase to the total of the dispersing phase and the binding phase being in a range of 72 to 90 percent by area and the average particle diameter being 1  $\mu\text{m}$  or less according to measurement of an electron microscopic texture; the dispersing phase of the cemented carbide cutting tool made of a tungsten carbide-based alloy comprises a dispersing phase composed of ultra-fine particles dispersed in a matrix and having a particle diameter of 100 nm or less, and the ultra-fine particles comprise a Co based alloy.

**13 Claims, No Drawings**

## CEMENTED CARBIDE CUTTING TOOL

## DETAILED DESCRIPTION OF THE INVENTION

## 1. Industrial Field of the Invention

The present invention relates to a cemented carbide cutting tool made of a tungsten carbide-based alloy having high chipping resistance (hereinafter referred to as a "cemented carbide cutting tool"), and more specifically, relates to a cemented carbide cutting tool having a sharp cutting edge and maintaining high cutting characteristics for long service life when used as an end mill having an intermittent cutting mode and when cutting is performed under heavy cutting conditions such as at high feed rate and high cutting depth.

## 2. Description of the Related Art

For example, Japanese Patent Application Laid-Open No. 3-43113 discloses a conventional cemented carbide cutting tool made of a tungsten carbide-based cemented carbide alloy (hereinafter referred to as a "cemented carbide alloy") composed of 8 to 13 percent by weight of Co and 0.1 to 3 percent by weight of Cr as constituents for forming a binding phase, the balance being tungsten carbide (hereinafter referred to as "WC") as a constituent for forming a dispersing phase, and incidental impurities, in which the rate of the dispersing phase to the total of the dispersing phase and the binding phase is in a range of 72 to 90 percent by area and the average particle diameter is 1  $\mu\text{m}$  or less according to measurement of an electron microscopic texture. Since the cemented carbide cutting tool has high toughness and high strength, it is known that the tool is used in practice as an end mill requiring such properties.

## 3. Problems to be solved by the Invention

In recent years, labor and energy saving for cutting tools has been eagerly awaited, and requirement for these cutting tools is towards heavy cutting conditions such as at high feed rate and high cutting depth. When the above conventional cemented carbide cutting tool is applied to an end mill used in an intermittent cutting mode under heavy cutting conditions, chipping (fine fracture) of the cutting edge occurs and thus the life is running out within a relatively short period.

## MEANS FOR SOLVING THE PROBLEMS

The present inventors have directed their attention to the above conventional cemented carbide cutting tool, have researched to improve chipping resistance, and have discovered the following. When using a powdered composite of WC and Co which is made by adding a distilled water containing dissolved cobalt nitrate as a Co source to a mixture of powdered tungsten oxide and powdered carbon in a predetermined ratio in place of powdered WC and powdered Co as raw powdered materials, followed by mixing and drying, and then performing, for example, reduction at 1,050° C. for 30 minutes in a nitrogen atmosphere and carbonization at 1,000° C. for 60 minutes in a hydrogen atmosphere, the dispersing phase of the cemented carbide alloy constituting the resulting cemented carbide cutting tool is composed of ultra-fine particles of a Co-based alloy having a particle diameter of 100 nm or less dispersed in a matrix. Thus, in the cemented carbide cutting tool, the constituents for forming a binding phase which includes major parts of a binding phase between the dispersing phases in the cemented carbide alloy becomes finer and more homogeneous compared to conventional cemented

carbide cutting tools having the same content of the constituents for forming the binding phase in the alloy. Based on recognition, in which a finer and more homogeneous distribution causes decreased thermal conductivity, the thermal conductivity was measured. This cemented carbide alloy for cutting tools has a thermal conductivity of 0.2 to 0.6 J/cm $\cdot$ sec $\cdot$ ° C. compared to 0.7 to 1.0 J/cm $\cdot$ sec $\cdot$ ° C. of a conventional cemented carbide alloy, and thus has superior chipping resistance when it is applied to an end mill used in intermittent cutting mode.

The present invention has been completed by the above, and is characterized by a cemented carbide cutting tool made of a tungsten carbide-based alloy having high chipping resistance comprising:

8 to 13 percent by weight of Co and 0.1 to 3 percent by weight of Cr as constituents for forming a binding phase, the balance being tungsten carbide as a constituent for forming a dispersing phase and incidental impurities, the rate of the dispersing phase to the total of the dispersing phase and the binding phase being in a range of 72 to 90 percent by area and the average particle diameter being 1  $\mu\text{m}$  or less according to measurement of an electron microscopic texture; wherein the dispersing phase of the cemented carbide cutting tool made of a tungsten carbide-based alloy comprises a dispersing phase composed of ultra-fine particles dispersed in a matrix and having a particle diameter of 100 nm or less, and the ultra-fine particles comprise a Co based alloy.

The Co content is limited to 8 to 13 percent by weight in the cemented carbide alloy constituting the cemented carbide cutting tool of the present invention, because sufficient toughness is not achieved at a content of less than 8 percent by weight whereas abrasion resistance steeply decreases at a content of higher than 13 percent by weight. The Cr content is also limited to 0.1 to 3 percent by weight, because the grain growth of the dispersing phase is insufficiently suppressed and thus the average diameter of the dispersing phase cannot be reduced to 1  $\mu\text{m}$  or less at a content of less than 0.1 percent by weight, whereas toughness significantly decreases at a content of higher than 3 percent by weight. Furthermore, high toughness is not achieved when the average particle diameter of the dispersing phase is larger than 1  $\mu\text{m}$ . As a result, Cr must be contained in an amount of 0.1 percent by weight or more while the average particle diameter of the powdered composite is maintained to 1  $\mu\text{m}$  or less, in order to control the average particle diameter of the dispersing phase to 1  $\mu\text{m}$  or less.

The diameter and the density of ultra-fine particles dispersed in WC are controlled by adjusting the average diameters of the powdered tungsten oxide and carbon which are used and by adjusting the conditions for reduction and carbonization. Since hardness and abrasion resistance unavoidably decrease if ultra-fine particles having a particle diameter higher than 100 nm are present in such a case, the diameter of the ultra-fine particles is limited to 100 nm or less.

The rate of the dispersing phase to the total of the dispersing phase and the binding phase is limited to a range of 72 to 90 percent by area, because desired abrasion resistance is not achieved at a rate of less than 72 percent whereas strength of the cemented carbide alloy decreased at a rate of higher than 90%.

## DESCRIPTION OF THE EMBODIMENTS

The cemented carbide cutting tool of the present invention will now be described in further detail with reference to examples.

Powdered  $\text{WO}_3$  with an average particle diameter of 0.6  $\mu\text{m}$ , powdered carbon with an average particle diameter of 0.4  $\mu\text{m}$ , and a mixed solvent composed of a distilled water containing a predetermined amount of dissolved cobalt nitrate  $[\text{Co}(\text{NO}_3)_2 \cdot 6\text{H}_2\text{O}]$  and a distilled water containing predetermined amounts of cobalt nitrate, and chromium nitrate  $[\text{Cr}(\text{NO}_3)_3]$  were prepared. These powdered  $\text{WO}_3$  and carbon and mixed solvent in a predetermined ratio were placed into a ball mill, wet-mixed for 72 hours, and dried. The mixture was subjected to reduction at 1,050° C. for 30 minutes in a nitrogen atmosphere and then carbonization at 1,000° C. for 60 minutes in a hydrogen atmosphere. Powdered composites A to J composed of WC and Co or composed of WC, Co and Cr having the formulations and average particle diameters shown in Table 1 were thereby prepared.

Powdered  $\text{Cr}_3\text{C}_2$  having an average particle diameter of 2.3  $\mu\text{m}$  was compounded in an amount shown in Table 2 with each of the powdered composites A to E. Each of the powdered composites A to J was pulverized by wet mixing for 72 hours in a ball mill, dried, and compacted under a pressure of 1 ton/cm<sup>2</sup> to form a green compact with a diameter of 13 mm and a length of 75 mm. The green compact was sintered at a predetermined temperature in a range of 1,380 to 1,480° C. for 1 hour in vacuo, and the sintered compact (cemented carbide alloy) was finished by grinding to form an end mill shape having a peripheral cutting edge with a diameter of 10 mm and a length of 70 mm. Cemented carbide cutting tools 1 to 10 in accordance with the present invention were thereby produced.

For comparison, conventional cemented carbide cutting tools 1 to 10 were produced under the same conditions, except for using powdered WC with an average particle diameter of 0.8  $\mu\text{m}$ , powdered  $\text{Cr}_3\text{C}_2$  with an average particle diameter of 2.3  $\mu\text{m}$ , and powdered Co with an average particle diameter of 1.2  $\mu\text{m}$  in the formulations shown in Table 2.

The Rockwell hardness (Scale A) and the thermal conductivity at room temperature in vacuo by a laser flash method of each of these cemented carbide cutting tools were measured, and the Co and Cr contents were measured. An arbitrary cross-section of each alloy was observed by a scanning electron microscope (SEM) to measure the ratio of the dispersing phase to the total of the dispersing phase and the binding phase, and to measure the average particle diameter of the dispersing phase. Whether or not ultra-fine particles were present in the dispersing phase was observed at a magnification of 350,000 $\times$  using a transmission electron microscope (TEM). When ultra-fine particles were present, the maximum particle diameter was measured and the major components thereof were identified using an energy dispersive X-ray spectrometer (EDS).

Each cemented carbide cutting tool (end mill) was subjected to a high-cutting-rate wet cutting test of steel under

the following conditions to measure the abrasion width of the peripheral edge:

Material to be cut: S45C (hardness (HB): 240)

Cutting speed: 60 m/min

Feed rate: 0.04 mm/tooth

Depth of cut in the axis direction: 15 mm

Depth of cut in the radial direction: 2 mm

Cut length: 15 m

The results are shown in Tables 3 and 4.

TABLE 1

| Type               | Average diameter ( $\mu\text{m}$ ) | Formulation (weight percent) |      |      |
|--------------------|------------------------------------|------------------------------|------|------|
|                    |                                    | Co                           | Cr   | WC   |
| Powdered Composite | A                                  | 1.0                          | 12.8 | —    |
|                    | B                                  | 0.9                          | 11.5 | —    |
|                    | C                                  | 0.8                          | 10.2 | —    |
|                    | D                                  | 0.8                          | 9.9  | —    |
|                    | E                                  | 0.7                          | 8.3  | —    |
|                    | F                                  | 0.8                          | 12.7 | 2.8  |
|                    | G                                  | 0.8                          | 12.2 | 1.5  |
|                    | H                                  | 0.7                          | 10.2 | 0.65 |
|                    | I                                  | 0.6                          | 10.0 | 0.60 |
|                    | J                                  | 0.5                          | 8.1  | 0.22 |

TABLE 2

| Type of cemented carbide cutting tool of | Formulation (weight %) | Type of conventional cemented carbide |          |         | Formulation |                         |    |
|------------------------------------------|------------------------|---------------------------------------|----------|---------|-------------|-------------------------|----|
|                                          |                        | this                                  | Powdered | carbide | WC          | $\text{Cr}_3\text{C}_2$ | Co |
| 1                                        | A: balance             | 3.0                                   | 1        | Balance | 3.0         | 13                      |    |
| 2                                        | B: balance             | 2.0                                   | 2        | Balance | 2.5         | 13                      |    |
| 3                                        | C: balance             | 0.8                                   | 3        | Balance | 2.0         | 12                      |    |
| 4                                        | D: balance             | 0.5                                   | 4        | Balance | 1.2         | 12                      |    |
| 5                                        | E: balance             | 0.2                                   | 5        | Balance | 0.8         | 10                      |    |
| 6                                        | F: 100                 | —                                     | 6        | Balance | 0.5         | 10                      |    |
| 7                                        | G: 100                 | —                                     | 7        | Balance | 1.0         | 9                       |    |
| 8                                        | H: 100                 | —                                     | 8        | Balance | 0.4         | 9                       |    |
| 9                                        | I: 100                 | —                                     | 9        | Balance | 0.2         | 8                       |    |
| 10                                       | J: 100                 | —                                     | 10       | Balance | 0.1         | 8                       |    |

TABLE 3

| Type of cemented carbide | Thermal conduction             |                                          | Co                          | Cr                 | Dispersing phase   |                | Ultra-fine particles               |                 |                       | Abrasion width of peripheral edge (mm) |
|--------------------------|--------------------------------|------------------------------------------|-----------------------------|--------------------|--------------------|----------------|------------------------------------|-----------------|-----------------------|----------------------------------------|
|                          | cutting tool of this invention | Hardness ( $\text{H}_\text{R}\text{A}$ ) | activity (J/cm · sec · °C.) | content (weight %) | content (weight %) | Ratio (area %) | Average diameter ( $\mu\text{m}$ ) | Observed or not | Maximum diameter (nm) |                                        |
| 1                        | 91.0                           | 0.35                                     | 12.4                        | 2.49               | 75.7               | 0.8            | Observed                           | 82              | Co                    | 0.40                                   |
| 2                        | 91.3                           | 0.41                                     | 11.2                        | 1.75               | 78.7               | 0.5            | Observed                           | 33              | Co                    | 0.42                                   |
| 3                        | 92.1                           | 0.40                                     | 10.0                        | 0.69               | 82.4               | 0.4            | Observed                           | 21              | Co                    | 0.35                                   |
| 4                        | 92.0                           | 0.52                                     | 9.8                         | 0.40               | 83.2               | 0.4            | Observed                           | 17              | Co                    | 0.33                                   |
| 5                        | 92.5                           | 0.37                                     | 8.2                         | 0.19               | 86.1               | 0.2            | Observed                           | 56              | Co                    | 0.29                                   |

TABLE 3-continued

| Type of cemented carbide       |                             | Thermal conductivity       | Co                 | Cr                 | Dispersing phase | Ultra-fine particles  |                 |                       | Abrasion        |                               |
|--------------------------------|-----------------------------|----------------------------|--------------------|--------------------|------------------|-----------------------|-----------------|-----------------------|-----------------|-------------------------------|
| cutting tool of this invention | Hardness (H <sub>RA</sub> ) | tivity (J/cm · sec · ° C.) | content (weight %) | content (weight %) | Ratio (area %)   | Average diameter (μm) | Observed or not | Maximum diameter (nm) | Major component | width of peripheral edge (mm) |
| 6                              | 91.1                        | 0.29                       | 12.6               | 2.80               | 75.0             | 0.5                   | Observed        | 77                    | Co              | 0.31                          |
| 7                              | 91.1                        | 0.33                       | 12.0               | 1.63               | 77.8             | 0.5                   | Observed        | 28                    | Co              | 0.31                          |
| 8                              | 92.3                        | 0.35                       | 10.1               | 0.66               | 82.3             | 0.4                   | Observed        | 36                    | Co              | 0.25                          |
| 9                              | 91.9                        | 0.44                       | 10.0               | 0.57               | 82.6             | 0.3                   | Observed        | 40                    | Co              | 0.30                          |
| 10                             | 92.4                        | 0.56                       | 8.0                | 0.19               | 86.5             | 0.2                   | Observed        | 50                    | Co              | 0.22                          |

TABLE 4

| Type of                                    |                             | Thermal conductivity       | Co                 | Cr                 | Dispersing phase | Ultra-fine particles  |                 |                       | Service life    |                                |
|--------------------------------------------|-----------------------------|----------------------------|--------------------|--------------------|------------------|-----------------------|-----------------|-----------------------|-----------------|--------------------------------|
| conventional cemented carbide cutting tool | Hardness (H <sub>RA</sub> ) | tivity (J/cm · sec · ° C.) | content (weight %) | content (weight %) | Ratio (area %)   | Average diameter (μm) | Observed or not | Maximum diameter (nm) | Major component | of peripheral edge by chipping |
| 1                                          | 90.8                        | 0.71                       | 12.9               | 2.60               | 74.4             | 0.9                   | Not obs.        | —                     | —               | 10 min.                        |
| 2                                          | 91.0                        | 0.78                       | 12.8               | 2.08               | 75.9             | 0.8                   | Not obs.        | —                     | —               | 12 min.                        |
| 3                                          | 91.1                        | 0.75                       | 11.9               | 1.72               | 77.8             | 0.6                   | Not obs.        | —                     | —               | 8 min.                         |
| 4                                          | 90.9                        | 0.73                       | 12.2               | 1.01               | 78.6             | 0.7                   | Not obs.        | —                     | —               | 6 min.                         |
| 5                                          | 91.9                        | 0.78                       | 10.1               | 0.69               | 82.2             | 0.6                   | Not obs.        | —                     | —               | 13 min.                        |
| 6                                          | 91.8                        | 0.82                       | 10.0               | 0.41               | 82.9             | 0.5                   | Not obs.        | —                     | —               | 15 min.                        |
| 7                                          | 92.3                        | 0.91                       | 8.8                | 0.85               | 83.9             | 0.3                   | Not obs.        | —                     | —               | 18 min.                        |
| 8                                          | 92.0                        | 0.85                       | 8.9                | 0.35               | 84.7             | 0.4                   | Not obs.        | —                     | —               | 17 min.                        |
| 9                                          | 92.2                        | 0.89                       | 8.0                | 0.18               | 86.4             | 0.4                   | Not obs.        | —                     | —               | 20 min.                        |
| 10                                         | 92.5                        | 0.95                       | 8.2                | 0.10               | 86.2             | 0.2                   | Not obs.        | —                     | —               | 20 min.                        |

## Advantage(s)

The results shown in Tables 3 and 4 demonstrate that the cemented carbide cutting tools 1 to 10 in accordance with the present invention have superior chipping resistance under high-cutting depth conditions of an end mill used in an intermittent cutting mode due to the presence of ultra-fine particles composed of a Co-based alloy having a particle diameter of 100 nm or less dispersed in a dispersing phase and due to a finer and more homogeneous distribution of the binding phase which is evaluated by a relatively low thermal conductivity. In contrast, the conventional cemented carbide cutting tools 1 to 10 have relatively short service lives due to low chipping resistance, although the hardness, the Co and Cr contents, the rate of the dispersing phase, and the average particle diameter are substantially the same as those in the cemented carbide cutting tools of the present invention.

As described above, the cemented carbide cutting tool of this invention has high chipping resistance and has superior cutting characteristics without chipping of the cutting edge for long periods under intermittent heavy cutting conditions such as at a high feed rate or a high cutting depth, in addition to continuous cutting conditions. Thus, the tool satisfactorily contributes to labor and energy saving in cutting operations.

What is claimed is:

1. A cemented carbide cutting tool made of a tungsten carbide-based alloy comprising:

a dispersing phase comprising tungsten carbide having an average particle diameter of 1 μm or less,

a binding phase comprising Co and Cr, and ultra-fine particles comprising a Co alloy having a particle diameter of 100 nm or less, wherein the dispersing phase is 72 to 90 percent by area of a cross section of the cemented carbide cutting tool; the ultra-fine particles are dispersed inside the tungsten carbide; and the cemented carbide cutting tool contains 8 to 13 percent by weight of Co, 0.1 to 3 percent by weight of Cr, the balance being tungsten carbide and incidental impurities.

2. The cemented carbide cutting tool of claim 1 prepared by:

mixing tungsten oxide powder, carbon powder, and an aqueous solution comprising cobalt and chromium; drying the resulting mixture; reducing the mixture; carbonizing the mixture; and sintering the mixture.

3. The cemented carbide cutting tool of claim 2 wherein said reducing is at 1050° C. in a nitrogen atmosphere.

4. The cemented carbide cutting tool of claim 2, wherein said carbonizing is at 1000° C. in a hydrogen atmosphere.

5. The cemented carbide cutting tool of claim 2, wherein said sintering is at 1380 to 1480° C. in a vacuum.

6. The cemented carbide cutting tool of claim 2 further comprising Cr<sub>3</sub>C<sub>2</sub>.

7. An end mill comprising the cemented carbide cutting tool of claim 2.

8. A process comprising:  
cutting a material with the cemented carbide cutting tool of claim 2.

9. The process of claim 8, wherein said material is steel.
10. The cemented carbide cutting tool of claim 1 further comprising  $\text{Cr}_3\text{C}_2$ .
11. An end mill comprising the cemented carbide cutting tool of claim 1.

12. A process comprising:  
cutting a material with the cemented carbide cutting tool  
of claim 1.
13. The process of claim 12, wherein said material is steel.

\* \* \* \* \*